# EUROPEAN PATENT SPECIFICATION

(11) **EP 4 294 981 B1**
(45) Date of publication and mention of the grant of the patent: **26.11.2025**
(21) Application number: 22735873.6
(22) Date of filing: 22.06.2022
(51) Int. Cl.: D21H 11/12, B65D 65/42, D21H 13/00, D21H 17/28, D21H 17/36, D21H 17/37, D21H 17/66, D21H 17/00, D21H 21/16, D21H 27/10, D21H 19/20

(54) **PAPER MATERIAL FOR FLUID CONTAINERS HAVING CHARACTERISTICS OF CALIBRATED FRAGILITY AND RIGIDITY AND A BARRIER PROPERTY**
PAPIERMATERIAL FÜR FLÜSSIGKEITSBEHÄLTER MIT KALIBRIERTEN ZERBRECHLICHKEITS- UND STEIFIGKEITSEIGENSCHAFTEN UND EINER BARRIEREEIGENSCHAFT
MATÉRIAU EN PAPIER POUR RÉCIPIENTS DE FLUIDE AYANT DES CARACTÉRISTIQUES DE FRAGILITÉ ET DE RIGIDITÉ CALIBRÉES ET UNE PROPRIÉTÉ DE BARRIÈRE

(30) Priority: 23.06.2021 IT 202100016493
(43) Date of publication of application: 27.12.2023
(73) Proprietor: FEDRIGONI S.P.A., 37135 Verona (IT)
(72) Inventor: MONACELLI, Luca, 33084 Cordenons (Pordenone) (IT)
(74) Representative: Modiano, Micaela Nadia
(86) International application number: PCT/EP2022/066962
(87) International publication number: WO 2022/268856

(56) References cited:
- WO-A2-2014/005697
- CA-A1- 2 439 354

## Description

The present invention relates to a paper material, a paper or paperboard produced with said paper material, a method of producing said paper material, and a container for fluid material produced with said paper material.

In the paper industry, there is a constant quest for new types of paper and paperboards for technical use having particular capacities and/or finishes, and above all intended as a barrier against gases and liquids, etc.

Paper-based products obtained with cellulose fibres and/or cotton and/or synthetic fibres, and with synthetic polymer-based and/or petroleum-derived additives, coupled or extruded with petroleum-derived polymers in order to contain and/or protect liquids and/or gels of varying nature, such as cosmetic or food products, have been present on the market for some time. For instance WO2014/005697A2 discloses a paper coated with a first surface coating comprising a polymer binder and an inorganic filler.

CA2439354A1 discloses a coated paperboard having barrier properties.

Such products cannot, however, be coupled with heat-sealable or gluable materials while maintaining the particular characteristics of rigidity and at the same time fragility necessary for a calibrated breakage of the container containing the gel and/or liquid of varying nature.

There is thus a perceived need to produce a paper material that may overcome the limits of the prior art.

The technical task of the present invention, therefore, is to provide a paper material of different grammages with a capability of being heat-sealable and couplable while maintaining the aforesaid properties of extreme rigidity, fragility and a capability of being cut with a neat, clean cut.

Yet a further object of the invention is to provide a paper material having properties of a barrier to water, fats, oils and gases without prejudicing adequate printability.

Another object of the invention is to provide a paper or paperboard produced with said paper material, a method of producing said paper material, and a container for fluid material produced with said paper material.

The technical task, as well as these and other objects, are achieved according to the present invention by providing a paper material, as defined in claim 4.

In the paper material said at least one polymeric substance is adapted to impart to the mixture of fibres mechanical strength and water resistance, said at least one inorganic filler is adapted to impart fragility, whilst the surface treated with at least one polyol and/or acrylic polymer and/or starch in addition to aluminium salts is adapted to impart properties of a barrier and resistance to fats, oils and gases.

Overall, the paper material has mechanical properties of rigidity, fragility and a capability of being cut and processed without losing fibrils of cellulose origin.

The present invention also relates to a container for fluid material,as defined in claim 1.

The present invention also relates to a method of producing said paper material, as defined in claim 5.

Other features of the present invention are defined, moreover, in the subsequent dependent claims, and in the claims related to the manufacturing method and to the device for use.

Additional features and advantages of the invention will become more apparent from the description of a preferred but not exclusive embodiment of the paper material according to the invention, illustrated hereinbelow by way of non limiting example.

The present invention relates to a velvety paper material (paper/paperboard) which, by virtue of a specially conceived mixture, a specific surface treatment and a production method has an extremely rigid, fragile structure and a capability of being neatly cut, without the typical releases of fibre.

Furthermore, the paper material of the invention is perfectly printable with an adequate print quality and makes it possible to obtain particular graphic effects that are difficult to obtain with traditional filtering paper materials.

In detail, the paper material of the invention comprises a base substrate comprising a mixture of cellulose fibres, cotton fibres and synthetic fibres, at least one polymeric substance, adapted to impart to the mixture of fibres mechanical strength (dry and wet) and water resistance, and at least one inorganic filler, adapted to impart to the material good characteristics of machinability, chemical stability and fragility, and aluminium salts in addition to at least one polyol and/or acrylic polymer and/or starch, adapted to impart a barrier property.

The base substrate has the following formulation:
- the mixture of cellulose fibres, cotton fibres and synthetic fibres, between 50% and 80% by weight
- the at least one polymeric substance, between 1% and 10% by weight
- the at least one inorganic filler, between 10% and 50% by weight
- the at least one polyol and/or acrylic polymer and/or starch, between 1% and 10% by weight
- the aluminium salts, between 1% and 30% by weight
said aluminium salts and said at least one polyol and/or acrylic polymer and/or starch being present in at least one outer surface of said outer shell.

The mixture of fibres comprises cellulose fibres and cotton fibres and synthetic fibres in a variable percentage proportion by weight: the length of the cellulose fibres is comprised between 0.2 mm and 5.0 mm; the content of cotton fibres and synthetic fibres in the mixture is in variable proportions of between 1% and 10% by weight.

The cellulose fibres comprise short and long bleached cellulose fibres, raw cellulose fibres and chemi-thermomechanical cellulose fibres in a mixture.

The synthetic fibres can preferably comprise an aliphatic polyolefin.

Preferably, the polymeric substance included in the base substrate comprises one or more resins based on colophony and/or alkyl ketene dimer and/or acetylsuccinic acid and/or epichlorohydrin and/or carboxymethylcellulose. Preferably, the inorganic filler is a mineral filler comprising one or more substances selected in the group consisting of carbonates, kaolins, talc and mixtures thereof.

Advantageously, the base substrate has at least one surface treated with at least one formula comprising a polyol and/or acrylic polymer and/or starch, in order to impart proprieties of a barrier to water, oils, greases and gases.

The surface treatment is for example an adhesive based on acrylic polymers, complex polyols, or products based on synthetic or natural waxes in order to impart proprieties of a barrier to water, oils, greases and gases.

More in detail, the following formulation was found to be suitable for the base substrate of the paper material:
- mixture of fibres between 60% and 70% by weight,
- the at least one polymeric substance, between 2% and 5% by weight
- the at least one inorganic filler, between 20% and 30% by weight
- the at least one polyol and/or acrylic polymer and/or starch, between 2% and 5% by weight
- the aluminium salts, between 1% and 5% by weight

In particular, the following formulation was found to be suitable for the base substrate of the paper material:
- cellulose fibres 60% by weight
- cotton fibres 0.2% by weight
- synthetic fibres 0.5% by weight
- epichlorohydrin-based resin 2% by weight
- carboxymethylcellulose-based resin 2% by weight
- calcium carbonate between 30% by weight
- aluminium salts 1% by weight
- styrene-acrylic latex 4% by weight.

The grammage of the paper material according to the present invention is comprised between about 50 g/sqm and 900 sqm.

The above-described paper material is produced in accordance with a further aspect of the present invention, with the following method.

The paper material is produced with a substantially known paper forming technique, for example on a continuous paper-making machine.

An aqueous mixture of cellulose fibres and first- or second-cut cotton fibres and synthetic fibres, containing the polymeric substance (resins based on colophony and/or alkyl ketene dimer and/or acetylsuccinic acid and/or epichlorohydrin and/or carboxymethylcellulose), and the inorganic mineral filler (carbonates, kaolins, talc and mixtures thereof), is prepared.

Subsequently, the water is removed from the mixture in order to form the base substrate of the paper material.

Then follows a step of treating the surface of one or both faces of the base substrate with an aqueous solution, for example composed of an aqueous solution of aluminium salts, polyol, and/or an acrylic adhesive or similar adhesives, in order to lend the necessary barrier property.

The method can subsequently comprise, after the surface treatment with the aqueous solution, a step of smoothing the paper wherein the base paper is smoothed to ISO 2494 Bendtsen smoothness values of less than about 800 ml/min.

The method also comprises a step of mechanically treating the base substrate to obtain a porosity of 1 sec to 50 sec according to the Gurley method.

Finally, the method can comprise a further step of mechanically treating the surface, in particular an embossing step.

Advantageously, a paper material produced in accordance with the present invention can be used to produce a container for fluid material.

In particular, the aforesaid paper material can be used as a replacement for a known plastic material as a substrate externally coupled to a shell for containing the fluid material.

The container for fluid material, be it a liquid or gel, advantageously has a substrate acting as an outer shell produced from the paper material described above.

Advantageously, the formulation that comprises the aluminium salts in addition to the adhesives is present at least in the outer surface of the outer shell.

The outer shell produced from this paper material is configured as a high-rigidity, high-fragility substrate and a barrier to water, oils, fats and gases.

The container thus comprises an inner plastic shell for containing the fluid material, wherein the inner shell is coupled, for example chemically applied, in particular glued or heat-sealed, to the outer shell.

## Claims

1. A container for fluid material, **characterized in that** it has an outer shell made of paper material comprising a base substrate having the following formulation:
- a mixture of cellulose fibers, cotton fibers and synthetic fibers comprising an aliphatic polyolefin, between 60% and 70% by weight, wherein the cellulose fibers comprise short and long bleached cellulose fibers, raw cellulose fibers and chemi-thermomechanical fibers in a mixture and wherein the length of the cellulose fibers is comprised between 0.2 mm and 5.0 mm and wherein the content of the cotton fibers and of the synthetic fibers in the mixture is in proportions varying between 1% and 50% by weight
- at least one polymeric substance, between 2% and 5% by weight, comprising one or more resins based on colophony, alkyl ketene dimer, acetylsuccinic acid, epichlorohydrin carboxymethylcellulose
at least one inorganic filler, between 20% and 30% by weight, wherein said at least one inorganic filler is a mineral filler and comprises one or more substances selected in the group consisting of carbonates, kaolins, talc and mixtures thereof
at least one polyol and/or acrylic polymer and/or starch, between 2% and 5% by weight aluminum salts, between 1% and 5% by weight
said aluminum salts and said at least one polyol and/or acrylic polymer and/or starch being present in at least an outer surface of said outer shell.

2. The container for fluid material according to any preceding claim, **characterized in that** the grammage of the paper material is comprised between 50 g/sqm and 900 sqm.

3. The container for fluid material according to any preceding claim, **characterized in that** it comprises an inner plastic shell for containing the fluid material, wherein the inner shell is coupled to the outer shell, which in turn acts as a substrate for the inner shell.

4. A paper material, **characterized in that** it comprises a base substrate having the following formulation:
- a mixture of cellulose fibers, cotton fibers and synthetic fibers comprising an aliphatic polyolefin, between 60% and 70% by weight, wherein the cellulose fibers comprise short and long bleached cellulose fibers, raw cellulose fibers and chemi-thermomechanical fibers in a mixture and wherein the length of the cellulose fibers is comprised between 0.2 mm and 5.0 mm and wherein the content of the cotton fibers and of the synthetic fibers in the mixture is in proportions varying between 1% and 50% by weight
- at least one polymeric substance, between 2% and 5% by weight, comprising one or more resins based on colophony, alkyl ketene dimer, acetylsuccinic acid, epichlorohydrin carboxymethylcellulose
at least one inorganic filler, between 20% and 30% by weight, wherein said at least one inorganic filler is a mineral filler and comprises one or more substances selected in the group consisting of carbonates, kaolins, talc and mixtures thereof
at least one polyol and/or acrylic polymer and/or starch, between 2% and 5% by weight aluminum salts, between 1% and 5% by weight
said aluminum salts and said at least one polyol and/or acrylic polymer and/or starch being present in at least one surface of said paper material.

5. A method of producing a paper material according to claim 4, **characterized in that** it comprises the steps of:
- preparing an aqueous mixture of said cellulose fibers, cotton fibers and synthetic fibers, said at least one polymeric substance, and said at least one inorganic filler;
- removing water from the mixture to form said base substrate of the paper material;
- carrying out a treatment of said at least one surface of said base substrate with at least one solution based on said aluminum salts and said at least one polyol and/or acrylic polymer.

6. The method according to the preceding claim, **characterized in that** said at least one polymeric substance included in said base substrate comprises one or more resins based on colophony and/or alkyl ketene dimer and/or acetylsuccinic acid and/or epichlorohydrin and/or carboxymethylcellulose, and said at least one inorganic filler is a mineral filler and comprises one or more substances selected in the group consisting of carbonates, kaolins, talc and mixtures thereof.

7. The method according to one or more of claims 5 and 6, **characterized in that**, after said surface treatment, a step of smoothing said base substrate is carried out, wherein said base substrate is smoothed to ISO 2494 Bendtsen smoothness values of less than about 800 ml/min.

8. The method according to one or more of claims 5-7, **characterized in that** it comprises a step of mechanically treating said base substrate to obtain a porosity of 1 sec to 50 sec according to the Gurley method.

## Patentansprüche

1. Ein Behälter für fluides Material, **dadurch gekennzeichnet, dass** es ein äußeres Gehäuse aus Papiermaterial hat, welches ein Basissubstrat mit folgender Formulierung umfasst:
- einer Mischung aus Zellulosefasern, Baumwollfasern und Synthetikfasern, die ein aliphatisches Polyolefin mit zwischen 60 und 70 Gewichtsprozent umfassen, wobei die Zellulosefasern kurze und lange gebleichte Zellulosefasern, rohe Zellulosefasern und chemo-thermomechanische Fasern in einer Mischung umfassen und wobei die Länge der Zellulosefasern zwischen 0,2 mm und 5,0mm beträgt und wobei der Gehalt an Baumwollfasern und Synthetikfasern in der Mischung in Anteilen vorliegt, die zwischen 1 Gewichtsprozent und 50 Gewichtsprozent variieren;
- mindestens einer polymeren Substanz mit zwischen 2 und 5 Gewichtsprozent, die ein oder mehrere Harze umfasst, basierend auf Kolophonium, Alkylketendimer, Acetylbernsteinsäure, Epichlorhydrincarboxymethylzellulose;
- mindestens einem anorganischen Füllstoff mit zwischen 20 und 30 Gewichtsprozent, wobei der mindestens eine anorganische Füllstoff ein mineralischer Füllstoff ist und eine oder mehrere Substanzen umfasst, gewählt aus der Gruppe bestehend aus Carbonaten, Kaolinen, Talk und Mischungen davon;
- mindestens einem Polyol und/oder Acrylpolymer und/oder Stärke mit zwischen 2 und 5 Gewichtsprozent;
- Aluminiumsalzen mit zwischen 1 und 5 Gewichtsprozent;
wobei die Aluminiumsalze und das mindestens eine Polyol und/oder Acrylpolymer und/oder die Stärke mindestens in einer äußeren Oberfläche des äußeren Gehäuses vorliegen.

2. Der Behälter für fluides Material gemäß einem beliebigen obigen Anspruch, **dadurch gekennzeichnet, dass** das Quadratmetergewicht des Papiermaterials zwischen 50 g/m² und 900m² beträgt.

3. Der Behälter für fluides Material gemäß einem beliebigen obigen Anspruch, **dadurch gekennzeichnet, dass** er ein inneres Kunststoffgehäuse zur Aufnahme des fluiden Materials umfasst, wobei das innere Gehäuse mit dem äußeren Gehäuse gekoppelt ist, welches wiederum als Substrat für das innere Gehäuse dient.

4. Ein Papiermaterial, **dadurch gekennzeichnet, dass** es ein Basissubstrat mit folgender Formulierung umfasst:
- einer Mischung aus Zellulosefasern, Baumwollfasern und Synthetikfasern, die ein aliphatisches Polyolefin mit zwischen 60 und 70 Gewichtsprozent umfassen, wobei die Zellulosefasern kurze und lange gebleichte Zellulosefasern, rohe Zellulosefasern und chemo-thermomechanische Fasern in einer Mischung umfassen und wobei die Länge der Zellulosefasern zwischen 0,2 mm und 5,0mm beträgt und wobei der Gehalt an Baumwollfasern und Synthetikfasern in der Mischung in Anteilen vorliegt, die zwischen 1 Gewichtsprozent und 50 Gewichtsprozent variieren;
- mindestens einer polymeren Substanz mit zwischen 2 und 5 Gewichtsprozent, die ein oder mehrere Harze umfasst, basierend auf Kolophonium, Alkylketendimer, Acetylbernsteinsäure, Epichlorhydrin Carboxymethylzellulose;
- mindestens einem anorganischen Füllstoff mit zwischen 20 und 30 Gewichtsprozent, wobei der mindestens eine anorganische Füllstoff ein mineralischer Füllstoff ist und eine oder mehrere Substanzen umfasst, gewählt aus der Gruppe bestehend aus Carbonaten, Kaolinen, Talk und Mischungen davon;
- mindestens einem Polyol und/oder Acrylpolymer und/oder Stärke mit zwischen 2 und 5 Gewichtsprozent;
- Aluminiumsalzen mit zwischen 1 und 5 Gewichtsprozent;
wobei die Aluminiumsalze und das mindestens eine Polyol und/oder Acrylpolymer und/oder die Stärke in mindestens einer Oberfläche des Papiermaterials vorliegen.

5. Ein Verfahren zur Herstellung eines Papiermaterials gemäß Anspruch 4, **dadurch gekennzeichnet, dass** es folgende Schritte umfasst:
- das Herstellen einer wässerigen Mischung aus den Zellulosefasern, Baumwollfasern und Synthetikfasern, der mindestens einen polymeren Substanz und dem mindestens einen anorganischen Füllstoff;
- das Entfernen von Wasser aus der Mischung, um das Basissubstrat des Papiermaterials zu bilden;
- das Durchführen einer Behandlung der mindestens einen Oberfläche des Basissubstrats mit mindestens einer Lösung, die auf den Aluminiumsalzen und dem mindestens einen Polyol und/oder Acrylpolymer basiert.

6. Das Verfahren gemäß dem obigen Anspruch, **dadurch gekennzeichnet, dass** die mindestens eine in das Basissubstrat eingeschlossene polymere Substanz ein oder mehrere Harze umfasst, die auf Kolophonium und/oder Alkylketendimer und/oder Acetylbernsteinsäure und/oder Epichlorhydrin und/oder Carboxymethylzellulose basieren und der mindestens eine anorganische Füllstoff ein mineralischer Füllstoff ist und eine oder mehrere Substanzen umfasst, gewählt aus der Gruppe bestehend aus Carbonaten, Kaolinen, Talk und Mischungen davon.

7. Das Verfahren gemäß einem oder mehreren der Ansprüche 5 und 6, **dadurch gekennzeichnet, dass** nach der Oberflächenbehandlung ein Schritt des Glättens des Basissubstrats durchgeführt wird, wobei das Basissubstrat auf einen ISO 2494-Bendtsen-Rauigkeitswert von weniger als ungefähr 800 ml/min geglättet wird.

8. Das Verfahren gemäß einem oder mehreren der Ansprüche 5-7, **dadurch gekennzeichnet, dass** es einen Schritt des mechanischen Behandelns des Basissubstrats, um eine Porosität von 1 sec bis 50 sec nach dem Gurley-Verfahren zu erhalten, umfasst.

## Revendications

1. Un récipient pour matière fluide, **caractérisé en ce qu'**il comporte une enveloppe extérieure en matériau papier comprenant un substrat de base ayant la formulation suivante:
- un mélange de fibres de cellulose, de fibres de coton et de fibres synthétiques comprenant une polyoléfine aliphatique, entre 60 % et 70 % en poids, dans lequel les fibres de cellulose comprennent des fibres de cellulose blanchies courtes et longues, des fibres de cellulose brutes et des fibres chimico-thermomécaniques en mélange, et dans lequel la longueur des fibres de cellulose est comprise entre 0,2 mm et 5, 0 mm, et dans lequel la teneur en fibres de coton et en fibres synthétiques dans le mélange est comprise entre 1 % et 50 % en poids
- au moins une substance polymère, comprise entre 2 % et 5 % en poids, comprenant une ou plusieurs résines à base de colophane, de dimère d'alkylcétène, d'acide acétylsuccinique, d'épichlorhydrine carboxyméthylcellulose
au moins une charge inorganique, comprise entre 20 % et 30 % en poids, où ladite au moins une charge inorganique est une charge minérale et comprend une ou plusieurs substances choisies dans le groupe constitué par les carbonates, les kaolins, le talc et leurs mélanges
au moins un polyol et/ou un polymère acrylique et/ou de l'amidon, compris entre 2 % et 5 % en poids
des sels d'aluminium, entre 1 % et 5 % en poids, lesdits sels d'aluminium et ledit au moins un polyol et/ou polymère acrylique et/ou amidon étant présents au moins sur une surface extérieure de ladite enveloppe extérieure.

2. Le récipient pour matière fluide selon l'une quelconque des revendications précédentes, **caractérisé en ce que** le grammage du matériau en papier est compris entre 50 g/m² et 900 m².

3. Le récipient pour matière fluide selon l'une quelconque des revendications précédentes, **caractérisé en ce qu'**il comprend une enveloppe intérieure en plastique destinée à contenir la matière fluide, dans lequel l'enveloppe intérieure est couplée à l'enveloppe extérieure, qui à son tour sert de substrat pour l'enveloppe intérieure.

4. Un matériau en papier, **caractérisé en ce qu'**il comprend un substrat de base ayant la formulation suivante :
- un mélange de fibres de cellulose, de fibres de coton et de fibres synthétiques comprenant une polyoléfine aliphatique, entre 60 % et 70 % en poids, dans lequel les fibres de cellulose comprennent des fibres de cellulose blanchies courtes et longues, des fibres de cellulose brutes et des fibres chimico-thermomécaniques en mélange et dans lequel la longueur des fibres de cellulose est comprise entre 0,2 mm et 5 mm, et dans lequel la teneur en fibres de coton et en fibres synthétiques dans le mélange est comprise entre 1 % et 50 % en poids
- au moins une substance polymère, comprise entre 2 % et 5 % en poids, comprenant une ou plusieurs résines à base de colophane, de dimère d'alkylcétène, d'acide acétylsuccinique, d'épichlorhydrine, carboxyméthylcellulose,
au moins une charge inorganique, comprise entre 20 % et 30 % en poids, où ladite au moins une charge inorganique est une charge minérale et comprend une ou plusieurs substances choisies dans le groupe constitué par les carbonates, les kaolins, le talc et leurs mélanges,
au moins un polyol et/ou un polymère acrylique et/ou de l'amidon, entre 2 % et 5 % en poids,
de sels d'aluminium, entre 1 % et 5 % en poids,
lesdits sels d'aluminium et ledit au moins un polyol et/ou polymère acrylique et/ou amidon étant présents dans au moins une surface dudit matériau en papier.

5. Un procédé de fabrication d'un matériau en papier selon la revendication 4, **caractérisé en ce qu'**il comprend les étapes consistant à:
- la préparation d'un mélange aqueux desdites fibres de cellulose, des fibres de coton et des fibres synthétiques, de ladite au moins une substance polymère et de ladite au moins une charge inorganique ;
- l'élimination de l'eau du mélange pour former ledit substrat de base du matériau en papier ;
- la réalisation d'un traitement de ladite au moins une surface dudit substrat de base avec au moins une solution à base desdits sels d'aluminium et dudit au moins un polyol et/ou polymère acrylique.

6. Le procédé selon la revendication précédente, **caractérisé en ce que** ladite au moins une substance polymère incluse dans ledit substrat de base comprend une ou plusieurs résines à base de colophane et/ou de dimère d'alkylcétène et/ou d'acide acétylsuccinique et/ou d'épichlorhydrine et/ou de carboxyméthylcellulose, et ladite au moins une charge inorganique est une charge minérale et comprend une ou plusieurs substances choisies dans le groupe constitué par les carbonates, les kaolins, le talc et leurs mélanges.

7. Procédé selon une ou plusieurs des revendications 5 et 6, **caractérisé en ce qu'**après ledit traitement de surface, une étape de lissage dudit substrat de base est effectuée, dans laquelle ledit substrat de base est lissé selon les valeurs de lissage Bendtsen ISO 2494 inférieures à environ 800 ml/min.

8. Procédé selon l'une ou plusieurs des revendications 5 à 7, **caractérisé en ce qu'**il comprend une étape de traitement mécanique dudit substrat de base pour obtenir une porosité de 1 seconde à 50 secondes selon la méthode Gurley.
